

Nov. 14, 1950

A. SOMMER

2,529,888

ELECTRON DISCHARGE DEVICE

Filed Feb. 25, 1948

FIG. 1.



FIG. 2.



Inventor

ALFRED SOMMER

By *Ralph E. Atherton*  
ATTORNEY

## UNITED STATES PATENT OFFICE

2,529,888

## ELECTRON DISCHARGE DEVICE

Alfred Sommer, Iver, England, assignor to Electric & Musical Industries Limited, Hayes, Middlesex, England, a company of Great Britain

Application February 25, 1948, Serial No. 10,941  
In Great Britain June 29, 1946

Section 1, Public Law 690, August 8, 1946  
Patent expires June 29, 1966

10 Claims. (Cl. 250—165)

1

This invention relates to the manufacture of electron discharge devices of the kind (hereinafter referred to as the kind described) having an electrode sensitised so as to be an emitter of photo-electrons or of secondary electrons (such electrons being in the claims generically referred to as impact electrons). Such devices comprise for example photo-electric cells and electron multipliers, and television transmission tubes employing photo-sensitive cathodes or photo-sensitive mosaic screens.

In one method of manufacturing such sensitive electrodes after the envelope of the device is evacuated and baked, a deposit of a suitable metal, such as antimony is applied and subsequently a sensitising substance such as caesium is admitted to react with the metal. It is found that considerably lower sensitivities are obtained if an antimony deposit is exposed to air prior to sensitisation compared with cases in which no exposure is allowed to occur.

For example, when the cathode of a photo-electric cell is made by depositing a layer of antimony after the final evacuation of the envelope, caesium being thereafter admitted to react with the antimony, the sensitivity of the cathode is usually between 50 and 100 microamperes per lumen of incident light. When however, the antimony deposit is exposed to air before the caesium sensitisation, considerably lower sensitivities are obtained, and in a series of tests it was found that after exposure of said deposit to air for a period of approximately 15 minutes, before sensitisation, the final sensitivity was under 20 microamperes per lumen. It is reasonable to assume that this deleterious effect results from superficial oxidation of the antimony deposit.

Now it is often desirable in manufacturing such devices to expose the deposit to air and it is therefore the object of this invention to enable such a deposit to be so exposed without such exposure seriously affecting the ultimate photo-electric sensitivity or secondary emission co-efficient of the electrode.

According to the invention there is provided a method of manufacturing an electron discharge device of the kind described wherein said sensitive electrode comprises a metal deposit which has been exposed to air, and wherein the deleterious effect of such exposure which would otherwise result is reduced or substantially eliminated by subjecting said deposit to a discharge in hydrogen and then without further exposure to air said deposit is sensitised in vacuo.

Preferably, said metal comprises antimony and the substance admitted to sensitise the metal comprises caesium, and in order to obtain the

2

most satisfactory results no baking of the device is effected after the discharge in hydrogen.

In order that the invention may be clearly understood and readily carried into effect, the same will now be described with reference to the accompanying drawing, wherein Figure 1 illustrates diagrammatically a fragment of an electrode for a photo-electric cell manufactured by a method according to one example of the present invention, and Figure 2 illustrates diagrammatically one stage of the method according to said example.

In the illustrated example of the invention applied to the manufacture of a photo-electric cell, 15 an antimony layer is deposited on a support 1 which is subsequently sealed into the envelope 2 of the cell to form a photo-electric cathode, during which operation the antimony layer is of course exposed to air. The envelope containing 20 the antimony layer is evacuated through an exhaust tube 3 and thereafter baked in vacuum at a temperature of between 250° C. and 300° C. and, after cooling, hydrogen is admitted by the tube 3 into the envelope of the cell until a suitable 25 pressure is achieved, the pressure being for example of the order of  $\frac{1}{10}$  of a millimeter of mercury. The antimony layer is then connected to the negative terminal of a voltage supply 4 and a suitable second electrode 5 within the envelope is connected to a point of positive potential to 30 cause a discharge to occur in the hydrogen. The potential difference required between said electrodes will depend upon a number of factors, among them the pressure in the envelope and may be for example 500 volts. This discharge 35 is maintained for a short time, for example one minute or less, and the hydrogen is then removed from the envelope by evacuation through the tube 3 and while maintaining the vacuum sensitisation is effected by admitting caesium to react 40 with the antimony, there being no further baking before said caesium sensitisation. The structure of the final electrode is indicated in Figure 1 wherein the reference numeral 6 indicates the layer of antimony sensitised with caesium, provided on the support 1.

Photo-electric cells manufactured by this method were found to have a sensitivity of over 50 microamperes per lumen so that harmful effects of exposing the antimony to air had been substantially avoided.

In a modification of the method described instead of applying a potential difference between the cathode and a second electrode in order to 55 cause the discharge in hydrogen to occur, the discharge is caused to occur by placing the device in a high frequency oscillatory field generated by means of a suitable high frequency oscillator.

The invention has been described as applied to the manufacture of photo-electric cells but it will be understood that it can also be applied to the manufacture of electron multipliers, having electrodes sensitised so as to be secondary electron emitters, and to the manufacture of television transmission tubes having photo-cathodes or photo-sensitive mosaic screens.

What I claim is:

1. A method of producing an electron discharge device having an electrode sensitised to be an emitter of impact electrons, including the steps of depositing metal under conditions involving exposure to air, subjecting the metal deposit to an electric discharge in hydrogen, whereby effects of exposure to air are reduced, and sensitising said deposit in vacuo before exposure to air.

2. A method of producing an electron discharge device comprising an evacuated envelope containing an electrode sensitised to be an emitter of impact electrons, including the steps of depositing metal on a support under conditions involving exposure to air, placing said support in an envelope, evacuating said envelope, admitting hydrogen to said envelope, establishing an electric discharge in said hydrogen to expose said metal deposit to the discharge, evacuating the hydrogen from said envelope, and sensitising said metal deposit in vacuo before exposure to air.

3. A method of producing an electron discharge device having an electrode sensitised to be an emitter of impact electrons, including the steps of depositing antimony under conditions involving exposure to air, subjecting the antimony deposit to an electric discharge in hydrogen to eliminate substantially deleterious effects of exposure to air, and exposing said deposit to caesium vapor in vacuo before exposure to air to sensitise the deposit.

4. A method of producing an electron discharge device comprising an evacuated envelope containing an electrode sensitised to be an emitter of impact electrons, including the steps of depositing antimony on an electrode support under conditions involving exposure to air, placing said support in an envelope, evacuating said envelope, admitting hydrogen to said envelope, establishing an electric discharge in the hydrogen to expose the antimony deposit to the discharge, evacuating hydrogen from said envelope, and admitting an alkali metal vapour to said envelope to sensitise said deposit before exposure to air.

5. A method of producing an electron discharge device comprising an evacuated envelope containing an electrode sensitised to be an emitter of impact electrons, including the steps of depositing antimony on a support outside an envelope, placing said support in the envelope, evacuating said envelope, admitting hydrogen to the envelope, establishing an electric discharge in the hydrogen to expose said antimony deposit to the discharge, evacuating hydrogen from said envelope, and admitting caesium vapour to said envelope to sensitise said antimony deposit before exposure to air.

6. A method of producing an electron discharge device comprising an envelope containing an electrode sensitised to be an emitter of electrons, including the steps of depositing metal on a support under conditions involving exposure to air, placing said support in an envelope, locating an electrode in said envelope and spaced from said support, evacuating said envelope, admitting hydrogen to said envelope, applying relatively

5 high and low potentials to said electrode and said deposit respectively to establish an electric discharge in said hydrogen, evacuating the hydrogen from said envelope, and sensitising said metal deposit in said envelope in vacuo before exposure to air.

7. A method of producing an electron discharge device comprising an evacuated envelope containing an electrode sensitised to be an emitter of impact electrons, including the steps of depositing antimony on a support under conditions involving exposure to air, placing said support in an envelope spaced from an electrode therein, evacuating said envelope, admitting hydrogen to said envelope, applying relatively high and low potentials to said electrode and said deposit respectively to establish an electric discharge in said hydrogen, evacuating the hydrogen from said envelope, and admitting caesium vapor to said envelope to sensitise said antimony deposit before exposure to air.

8. A method of producing an electron discharge device comprising an envelope containing an electrode sensitised to be an emitter of impact electrons, including the steps of depositing metal on a support under conditions involving exposure to air, placing said support in an envelope, evacuating said envelope, admitting hydrogen to said envelope, producing a high frequency oscillatory field in the region of said envelope to cause an electric discharge in the envelope in the presence of the hydrogen, evacuating the hydrogen from the envelope, and sensitising the metal deposit in said envelope in vacuo before exposure to air.

9. A method of producing an electron discharge device comprising an evacuated envelope containing an electrode sensitised to be an emitter of impact electrons, including the steps of depositing antimony on a support under conditions involving exposure to air, locating said support in an envelope, evacuating said envelope, admitting hydrogen to said envelope, producing a high frequency oscillatory field in the region of said envelope to cause an electric discharge in the envelope in the presence of the hydrogen, evacuating the hydrogen from the envelope, and admitting caesium vapour to said envelope to sensitise said antimony deposit before exposure to air.

10. A method of producing an electron discharge device comprising an evacuated envelope containing an electrode sensitised to be an emitter of impact electrons, including the steps of depositing antimony on a support under conditions involving exposure to air, locating said support in an envelope, evacuating said envelope, admitting hydrogen to said envelope, establishing an electric discharge in the hydrogen to expose said antimony deposit to the discharge, evacuating hydrogen from the unbaked envelope, and admitting alkali metal vapour to said envelope to sensitise said antimony deposit before exposure to air.

ALFRED SOMMER.

#### REFERENCES CITED

The following references are of record in the file of this patent:

#### UNITED STATES PATENTS

| Number    | Name           | Date          |
|-----------|----------------|---------------|
| 2,045,637 | de Boer et al. | June 30, 1936 |
| 2,285,058 | Samson         | June 2, 1942  |
| 2,401,737 | Janes          | June 11, 1946 |